

## UNITED STATES PATENT OFFICE

HARRY H. ALEXANDER, OF WESTFIELD, NEW JERSEY

## REFINING OF COPPER

No Drawing.

Application filed July 5, 1928. Serial No. 290,703.

This invention relates to the metallurgy of copper and has for its object the provision of improvements in the method of refining copper. The invention more particularly contemplates the desulfurization of copper contaminated with sulfur and/or its compounds and the like.

Crude or partially refined copper—such as pig copper or cathodes from electrolytic plants, is usually contaminated with appreciable amounts of sulfur and/or its compounds, as well as with other well known impurities. In the furnace refining of copper as heretofore more generally practiced, the metal and its impurities are melted. The molten material is suitably aerated to oxidize the impurities, some of which pass off as vapors and gases, while others pass into the slag forming on the top of the molten copper. In the case of sulfur and/or its compounds, the sulfur is in part volatilized and in part converted to sulfur dioxide which passes off as a gas.

The aeration of the molten material is effected in various ways. The older method is to flap the top surface of the molten material with a rabble, while admitting air into the refining furnace, in order to subject the impurities to the oxidizing effect of the air. A later method is to pass air, under pressure, into the body of molten material. The removal of sulfur and/or its compounds is accomplished with considerable difficulty, and a large excess of air must therefore be employed in the refining operation. Both methods have the desirable effect of oxidizing impurities, but the very undesirable effect of also oxidizing appreciable amounts of the copper—frequently as much as 6%.

The oxidized copper must then be subjected to a deoxidizing or reducing operation to obtain a relatively pure copper product. This latter refining or reducing operation is conducted in various ways, generally by the introduction into the body of molten copper of a suitable reducing agent, such as wooden poles or carbonaceous materials.

In the case of the usual copper to be refined, the removable impurities other than sulfur will pass out of the aerated copper

bath in about two hours. The end of this stage of the refining operation may be determined by noting when the formation of slag appears to cease. About two hours more aeration are required to drive out the sulfur. 55

As a result of my investigations I have determined that the aeration or scorification action may advantageously be terminated before the conversion of appreciable amounts of copper to copper oxide has taken place. 60 The removable impurities present in the molten copper not oxidized or removed by the air treatment may be suitably removed in accordance with the practice of my invention. 65

In the practice of the present invention, copper contaminated with sulfur and/or its compounds and the like may be refined without oxidizing the copper, and the customary deoxidizing or reducing step may therefore 70 be avoided. Or, the invention may be practiced in such a way as to desulfurize the copper while oxidizing some of the copper, but at a material saving in time over what the prior practice requires. 75

According to my invention, a body of molten copper contaminated with sulfur and/or its compounds, hereafter to be referred to as sulfur, and the like is subjected to the action of steam, preferably dry steam 80 under pressure, whereby the copper is desulfurized.

Steam at the temperatures employed has the advantage of not oxidizing the molten copper, while at the same time oxidizing the 85 sulfur to form sulfur dioxide gas. Steam, moreover, tends to drive out residual sulfur, as well as other removable impurities present in the copper bath. The steam is preferably superheated in order to dry the same. 90

When the contaminating sulfur is present as copper sulfide, the reaction results in the formation of copper and sulfur dioxide gas, in accordance with the reaction:



This reaction, moreover, has the advantage of forming free hydrogen which has the capacity for taking up free oxygen that may be present above the copper to be refined. So 100

long as the reaction takes place and hydrogen is being evolved, this free oxygen present above the copper cannot exercise an oxidizing effect on the copper. Hence, the formation of copper oxide is prevented. The prevention of the formation of copper oxide can be conducted in this manner, however, only so long as there is sufficient sulfur to keep on generating hydrogen until all of the free oxygen has been taken up. In case the above reaction goes to completion, any free oxygen that has not been taken up by the hydrogen becomes available as an oxidizing agent for the copper. Copper oxide then results.

15 This situation applies with equal force to the gaseous condition maintained above the copper bath. Even though the formation of copper oxide should be prevented within the copper bath, the maintenance of oxidizing 20 conditions above the bath will result in the formation of copper oxide. This may or may not be avoided, as desired.

15 The invention may be practiced in various ways. Thus, the molten copper within the refining furnace may first be subjected to the usual air blast or babbling operation in order to oxidize substantially all of the impurities. That is to say, the aeration or scorification treatment may be conducted until all 30 of the removable impurities, except some sulfur, have been taken out of the copper bath. The introduction of air is terminated at that point, which may be determined by observing when the formation of slag begins to 35 cease. The copper bath will still contain appreciable amounts of sulfur. Instead of removing this sulfur by employing an excess of air, the copper is preferably subjected to the steam treatment of the invention. The action 40 of the steam is to cleanse the copper of the sulfur, while at the same time inhibiting the oxidation of copper, particularly when a non-oxidizing atmosphere is maintained over the copper bath.

45 Another procedure is to subject the molten material in the refining furnace to the steam treatment of the invention in order to take out all such impurities as are removable by steam at the temperatures employed. Moreover, the steam treatment may be conducted until the sulfur has been removed. The desulfurized copper bath may then be subjected, if necessary, to the usual air blast in order to remove any remaining impurities. In this 55 manner, the oxidation of copper may be kept down to a minimum, particularly if a non-oxidizing atmosphere is again maintained above the copper bath.

60 It will, of course, also be apparent that the use of steam and the use of air may be alternated, as seen fit in the refining operation. In some instances, the refining operation may also lend itself to the practice of subjecting both steam and air, separately but simultaneously, or a mixture of steam and air, into the

copper bath. Such a procedure may be particularly advantageous if it is desired to materially decrease the time for performing the refining operation, and where there is no particular concern as to the production of a final 70 copper product that is relatively free of copper oxide. Various other modifications of the practice of the invention may, of course, be resorted to, but it is to be understood that the omission of a discussion of them is not to 75 be regarded as otherwise restrictive of the scope of the invention.

75 The apparatus usually employed to inject air into copper refining furnaces may advantageously be employed for the introduction 80 of steam into the metal bath. In order that a thorough distribution of the steam may be effected throughout the body of the molten material, it is advisable to introduce steam into the molten bath at a plurality of points, 85 preferably near the bottom of the refining furnace. Since it is preferred to use dry steam, the pipes leading from the source of steam to the refining furnace should be insulated to minimize condensation of steam. 90 Special injectors may, of course, be provided for steam alone.

95 In case it is desired to inhibit the formation of copper oxide, the openings leading into the furnace should be tightly closed to prevent the ingress of air. In other words, a non-oxidizing atmosphere should be provided above the metal bath. Reducing gases may of course be maintained above the metal bath. A molten protecting cover, such as 100 described and claimed in my copending application, Serial No. 123,886, filed July 21, 1926, of which this application is a continuation in part, may advantageously be employed to protect the molten bath from oxidizing 105 influences during the steaming treatment. According to said copending application a molten protective cover is contemplated that consists at least in part of soda glass having a melting point not higher, and preferably 110 lower, than that of the copper.

115 In case it is not desired to inhibit the formation of copper oxide, an oxidizing atmosphere may, of course, be maintained above the metal bath. The highly heated molten copper at the top of the metal bath then contacts with the oxygen of the air and copper oxide is formed. The use of steam instead of air, particularly at the end of the refining operation, is nevertheless advantageously resorted to in order to drive out the sulfur. Even though copper oxide has been formed, the time of the refining operation will be materially reduced over that heretofore generally required.

120 Even in the case of desulfurization with air, some of the sulfur dioxide gases tend to be occluded in, or are retained by, the molten copper. When an excessive amount of air is made to rise through the body of molten cop- 130

per to remove such sulfur gases, a further opportunity is of course given for the molten copper to be oxidized. The use of steam, on the other hand, not only inhibits the formation of copper oxide, but also effectively drives out these sulfur dioxide gases.

It will thus be seen that in the practice of this invention, it is possible to effectively remove the chief impurity of copper, sulfur, without oxidizing the copper, or at least oxidizing a minimum of copper if that is desirable. The practice of the invention, moreover, has the advantage of removing other impurities. In the instances where it is not desired to inhibit the formation of copper oxide, the refining operation contemplated by the invention may be conducted in much less time, thereby effecting a very important economy.

20 I claim:

1. The method of refining copper which comprises maintaining a substantially non-oxidizing atmosphere above the copper in the form of a molten bath while subjecting the molten copper to the action of steam under pressure, said steam being introduced into the body of molten copper, whereby the copper is desulfurized and the formation of copper oxide is inhibited.

20 2. The method of refining copper containing an appreciable amount of sulfur as at least one of the contaminating impurities, which comprises aerating the copper while in a molten state, said aerating operation being continued until the formation of slag ceases, and then introducing steam under pressure into the body of molten copper to complete the refining operation.

3. The method of refining copper which comprises maintaining a molten protective cover consisting at least in part of soda glass having a melting point not higher than that of the copper over the copper bath, and introducing steam under pressure into the body of molten copper.

4. The method of refining copper which comprises aerating the molten copper partially to remove impurities, maintaining a molten protective cover consisting at least in part of soda glass having a melting point not higher than that of the copper over the partially refined copper, and then introducing steam under pressure into the body of molten copper.

5. The method of refining copper which comprises aerating molten copper partially to remove impurities, then providing a substantially non-oxidizing atmosphere above the copper bath, and introducing steam under pressure into the body of molten copper.

6. The method of refining copper containing sulfur as at least one of the contaminants which comprises maintaining an oxidizing atmosphere over the copper bath, introducing steam under pressure into the body of

molten copper until only a relatively small amount of sulfur remains, then providing a substantially non-oxidizing atmosphere over the copper bath, and introducing further amounts of steam under pressure into the body of partially refined copper to complete the refining operation.

7. The method of refining copper containing an appreciable amount of sulfur as at least one of the contaminating impurities which comprises substantially sealing the furnace in which the refining operation is conducted against the seepage of outside air, and subjecting the copper in the form of a molten bath to the action of steam under pressure whereby the copper is desulphurized and the formation of copper oxide is inhibited.

8. The method of refining copper containing sulfur as at least one of the contaminants which comprises maintaining an oxidizing atmosphere over the copper bath by permitting the seepage of outside air into the furnace in which the refining operation is conducted, introducing steam under pressure into the body of molten copper until only a relatively small amount of sulfur remains, then providing a substantially non-oxidizing atmosphere over the copper bath by sealing the furnace against the entrance of outside air, and introducing further amounts of steam under pressure into the body of partially refined copper to complete the refining operation.

In testimony whereof I affix my signature. 100  
HARRY H. ALEXANDER.

105

115

120

125

130